

# UNITED STATES PATENT OFFICE.

EUGENE H. COWLES AND ALFRED H. COWLES, OF CLEVELAND, OHIO.

## ALLOY.

SPECIFICATION forming part of Letters Patent No. 397,699, dated February 12, 1889.

Application filed July 8, 1885. Serial No. 171,011. (No specimens.)

*To all whom it may concern:*

Be it known that we, EUGENE H. COWLES and ALFRED H. COWLES, citizen of the United States, residing at Cleveland, in the county of 5 Cuyahoga and State of Ohio, have invented certain new and useful Improvements in Alloys; and we do hereby declare the following to be a full, clear, and exact description of the invention, such as will enable others skilled in the 10 art to which it appertains to make and use the same.

This invention relates to metallic alloys; and it consists in the combination of the metals hereinafter specified.

15 In carrying out our invention we take of—

|                 | Parts.       |
|-----------------|--------------|
| Copper .....    | 63.333       |
| Nickel .....    | 33.333       |
| Aluminium ..... | 3.333        |
|                 | <hr/> 99.999 |

These we fuse together in a crucible, so that they may be thoroughly mixed and alloyed.

In order to secure the best possible result 25 and prevent the formation of oxides, powdered carbon or common salt may be spread over the metals in the crucible, so as to cover them and exclude the air. The resulting alloy is a new compound, which we have chosen to designate "Hercules metal" on account of its 30 great strength, toughness, and resilience. This metal is the strongest known to the arts, and castings of it average over one hundred thousand pounds to the square inch in tensile 35 strength, which is considerably more than the best grades of iron or steel.

The proportions of the various metals we have given to form the alloy are those which are found to give the best results in practice. 40 These proportions may be materially varied without seriously impairing the strength or usefulness of the alloy; but to secure the

greatest strength, elasticity, and hardness it is necessary that each of the metals—copper, nickel, and aluminium—should be perfectly 45 pure and free from impurities, and that no other ingredient should be added to them either before or while in a state of fusion. The alloy when thus prepared and free from impurities compares favorably in hardness 50 with the best tempered steel. It is also untarnishable, and is not affected by sulphur or acids to any appreciable extent. These peculiar properties render it specially adapted as a material from which table-cutlery and similar articles may be manufactured. 55

We are aware that it is not broadly new to make an alloy containing copper, nickel, and aluminium, an alloy containing these metals having been formed of which ninety-one per 60 cent. was copper. The remaining metals were, however, impure. They were used in such small quantity that the alloy did not possess the characteristic strength and hardness of the alloy hereinbefore described, and had the 65 quantity of nickel and aluminium been increased the impurities contained in them would have prevented the alloy from having any value or utility.

Having thus fully described our invention, 70 what we claim as new, and desire to secure by Letters Patent, is—

A metallic alloy consisting of a proportion of copper, nickel in about half the proportion of the copper, and a percentage of aluminium, 75 substantially as set forth.

In testimony whereof we affix our signatures in presence of two witnesses.

EUGENE H. COWLES.  
ALFRED H. COWLES.

Witnesses:

B. O. WILCOX,  
ROBT. F. SCHADE.